

A. J. TOWNSEND AND H. M. NAUGLE.  
PRESSED STEEL MACHINE PARTS AND METHOD OF MAKING THE SAME.  
APPLICATION FILED MAR. 24, 1919.  
**1,317,055.** Patented Sept. 23, 1919.  
4 SHEETS—SHEET 1.

*Fig. 1.*



*Fig. 2.*



*Fig. 3.*



INVENTORS

Arthur J. Townsend *et al*  
Harry M. Naugle.  
Frease, Merle, Saywell *et al*/Bond

ATTORNEYS

A. J. TOWNSEND AND H. M. NAUGLE.  
PRESSED STEEL MACHINE PARTS AND METHOD OF MAKING THE SAME.  
APPLICATION FILED MAR. 24, 1919.

1,317,055.

Patented Sept. 23, 1919.  
4 SHEETS—SHEET 2.



INVENTORS  
Arthur J. Townsend *et al.*  
Harry M. Naugle.

Frease, Minkel, Saywell *et al.* Bond  
ATTORNEYS.

A. J. TOWNSEND AND H. M. NAUGLE,  
PRESSED STEEL MACHINE PARTS AND METHOD OF MAKING THE SAME.

APPLICATION FILED MAR. 24, 1919.

1,317,055.

Patented Sept. 23 1919.

4 SHEETS—SHEET 2

*Fig. 13.*



*Fig. 14.*



*Fig. 15.*



INVENTORS

Arthur J. Townsend &  
Harry M. Naugle.

Frease, Merkel, Saywell and Bond

ATTORNEYS.

A. J. TOWNSEND AND H. M. NAUGLE.

PRESSED STEEL MACHINE PARTS AND METHOD OF MAKING THE SAME.

APPLICATION FILED MAR. 24, 1919.

1,317,055.

Patented Sept. 23, 1919.

4 SHEETS—SHEET 4.



INVENTORS

Arthur J. Townsend

Harry M. Naugle.

Frease, Merkel, Saywell and Bond

ATTORNEYS

# UNITED STATES PATENT OFFICE.

ARTHUR J. TOWNSEND AND HARRY M. NAUGLE, OF CANTON, OHIO.

PRESSED-STEEL MACHINE PARTS AND METHOD OF MAKING THE SAME.

1,317,055.

Specification of Letters Patent. Patented Sept. 23, 1919.

Application filed March 24, 1919. Serial No. 284,540.

To all whom it may concern:

Be it known that we, ARTHUR J. TOWNSEND and HARRY M. NAUGLE, both citizens of the United States, both residing at Canton, 5 in the county of Stark and State of Ohio, have invented certain new and useful Improvements in Pressed-Steel Machine Parts and Methods of Making the Same, of which the following is a specification, and which 10 are illustrated in the accompanying drawings, forming a part thereof.

The invention relates to machine parts, meaning thereby the movable parts of machinery which must have hardness to resist 15 wear in addition to the strength and toughness required to withstand shocks and to transmit force or support weight and the invention is more especially concerned with those machine parts which are desirably 20 made in the lightest possible form consistent with strength, such for example, as the hollow piston pins of internal combustion engines, brake drums for automobiles, wheel hubs and the like. In the commercial manu- 25 facture of these parts it has been customary to employ one or the other of two methods of production both of which comprise the formation of the parts to substantially finished dimensions from mild steel or steel al- 30 loys and the subsequent case hardening of those surfaces of the parts which are ex- posed to wear in use. One of the methods of production so employed involves cutting 35 the parts from solid or only partially formed blocks or bars, while in the other of these 40 methods the parts are cold pressed or drawn to shape from plates or disks of predeter- mined dimensions. In the one case, a sub- 45 stantial part of the weight of the metal, frequently more than is retained in the finished article is removed and lost and sometimes, as in making a hollow piston pin, for 50 example, the part removed comprises the dense interior portion of the metal while the 55 part retained is that most likely to be defective because of surface cracks or the like and great difficulty is experienced in cutting the interior wall exactly concentric with the exterior surface to obtain the highly desirable 60 symmetrical distribution of weight in the finished article. The shaping of the articles by the cold pressing or drawing method, on the other hand, usually requires a consider- 65 able number of partial operations or steps 70 and careful annealing of the metal for each 75 of these steps.

It will thus be understood that both of the said methods of forming the articles are expensive and that they are commercially practicable only when steel or steel 60 alloys containing very little carbon are used. Furthermore, as these low carbon steels and steel alloys are not susceptible of being ap- 65 preciably hardened by heat treatment, the subsequent case hardening of the parts, here- 70 fore mentioned, is always required. This case hardening of the parts frequently fails to obtain uniform hardness throughout the wearing surfaces and the parts are weakened rather than strengthened by this treatment. 75

The object of the present invention is the provision of machine parts of the kind de- 80 scribed of reduced weight but of equal or greater strength and durability and of more uniform and improved hardness, and a 85 method of producing the same: To this end the invention contemplates the selection of plates or the like of steel or steel alloy con- 90 taining sufficient carbon to respond to hard- ening by heat treatment in a marked degree, heating the said plates to a temperature at 95 which they are readily ductile, pressing the same while hot between dies to the shape and substantially finished dimensions of the ar- 100 ticles desired, but preferably maintaining a like thickness with the original plates, smoothing the wearing surfaces of the ar- 105 ticles and then hardening the articles through- out by appropriate heat treatment in ac- cordance with the analysis of the selected 110 steel or steel alloy. In the use of steel alloys which are too hard to be machined when cooled in the air from a working tempera- 115 ture, the smoothing of the wearing surfaces of the articles is permitted without reheat- 120 ing the articles for annealing, if the original cooling is substantially retarded, as by pack- 125 ing the articles in lime immediately upon their removal from the forming dies. 130

In the accompanying drawings:— 135

Figure 1 is a central sectional view of a 140 brake drum formed of medium or high car- 145 bon steel or steel alloy and made in accord- 150 ance with the present invention, and for 155 comparison—

Fig. 2 is a similar view of a brake drum 160 formed of mild or low carbon steel by the 165 cold pressing process heretofore used, and

Fig. 3 is a sectional view of a forging for 170 a brake drum, as heretofore employed, the 175 form of the finished brake drum being shown in dotted lines, 180

Fig. 4 is a blank of medium or high carbon steel or steel alloy of the proper size and shape to be formed into a hollow piston pin in accordance with the present invention,

5 Figs. 5 and 6 show the product after successive operations of the present method to form the said piston pin from the blank illustrated in Fig. 4, and for comparison—

Fig. 7 is similar to Fig. 4 but shows a blank of mild or low carbon steel of proper size and shape to be formed into a hollow piston pin by the cold pressing method herefore used, and

15 Figs. 8, 9, 10, 11 and 12 show the product after successive operations by the said cold pressing process to form the piston pin from the blank shown in Fig. 7.

Fig. 13 is a view, partly in section and partly in side elevation, showing dies for 20 performing the first operation of producing a hub by the present method, a blank of steel of the character above mentioned in the brief description of Figs. 1 and 4, being in the die,

Fig. 14 is similar to Fig. 13 but shows the dies in closed position upon the work,

Fig. 15 is similar to Fig. 14 but shows the dies employed in a further step in the operation of producing the said hub by the present method, and for comparison with Figs.

30 13, 14 and 15,  
Fig. 16 is a view, partly in section and  
partly in side elevation, showing dies for  
performing the first operation of producing  
a hub by the cold pressing method hereto-  
35 fore used, a blank of mild steel being shown  
in the die.

Fig. 17 is similar to Fig. 16 and shows the same dies in closed position upon the work,

40 Figs. 18, 19 and 20 are each similar to Fig. 17 but show the dies used to perform the several additional operations necessary to produce the finished shape of the hub, by the cold pressing process,

Fig. 21 is a detail sectional view greatly enlarged and conventionally representing the uniform texture of a medium or high carbon steel or steel alloy after the same has been hardened by heat treatment, and for comparison—

Fig. 22 is similar to Fig. 21 but shows, in like conventional manner, the texture of a mild or low carbon steel after the same has been carbonized or case hardened.

In carrying out the invention the selected blank, as 11 (Fig. 4) or 28 (Fig. 18) will usually be a relatively thin circular disk of steel which may have a medium carbon content of approximately .45%. In the annealed state and when alloyed with approximately one per cent. of chromium this steel has physical properties substantially as follows:—

|                                      |       |
|--------------------------------------|-------|
| Elastic limit pounds per square inch | 55000 |
| Reduction of area                    | 35%   |
| 65 Elongation in two inches          | 25%   |

For the production of a hollow piston pin, as 13, (Fig. 6) the blank 11 is heated to a working temperature which is preferably maintained between  $1500^{\circ}$  and  $1700^{\circ}$  F. to secure the desired ductility without excessive scaling. While so heated, the blank is pressed between appropriate dies to the required size and shape, a single intermediate shape, as 12 (Fig. 5) being usually sufficient and the entire pressing operation being ordinarily performed without reheating. In event an alloy steel has been used for the blank 11 and it is desired to smooth the wearing surface of the article with a cutting tool, cooling from the working temperature is preferably retarded by packing the article in lime, thus annealing the same; and by quickly performing the reduced number of pressing operations, such subsequent annealing as well as the pressing of the article, may be accomplished by a single heating of the same. In the case of the piston pin 13 the closed end may then be removed by cutting through the article at the place indicated by the dotted line 14 (Fig. 6) without further annealing. If so-called straight carbon steel has been used for the blank, as 11, the article may be allowed to cool in the air after being pressed to shape.

Whether formed from straight carbon or 95 alloy steel, the article, as 13, after being trimmed as indicated, and after having had its wearing surface smoothed, when required, is hardened by heat treatment and polished. The finished article will thus be 100 hard and tough throughout as conventionally represented at 35 (Fig. 21). As an example illustrating the invention it has been found that when an alloy steel containing approximately .45% carbon and one per cent. 105 chromium is used, the physical properties of the finished article are substantially as follows:

|                                         |         |     |
|-----------------------------------------|---------|-----|
| Elastic limit pounds per square<br>inch | 200,000 | 110 |
| Reduction of area                       |         | 10% |
| Elongation of two inches                |         | 8%  |

While the heat treatment for hardening the article, as 13, and the resulting physical properties may vary somewhat with the analysis of the selected steel, the said heat treatment will generally comprise quenching in oil from a temperature above that of decalescence and reheating to a lower temperature for the purpose of removing cooling strains and modifying the intense hardness produced by quenching. 115 120

By the method just described the number of operations necessary in stamping or 125 pressing any article is reduced, at least one-half, in comparison with the cold pressing method heretofore used. Figs. 7 to 12 inclusive show the operations necessary with the cold pressing process to form a piston 130

pin from mild or low carbon steel. The blank from which the pin is stamped is shown at 5, and represents a blank of mild steel of proper size and shape to form the 5 pin. By successive stamping operations upon suitable dies this blank assumes the forms shown at 6, 7, 8 and 9 and after each 10 pressing operation the product is annealed before the next pressing operation. After 15 the product has passed through all of the necessary stamping operations and assumes the form shown at 9 (Fig. 12) the closed end of the product is cut off as indicated by the dotted line 10 and the pin is carbonized or case hardened, giving it a thin hardened shell upon its surface while the interior 20 of the steel remains soft.

In Fig. 22 the thin hardened shell of a 25 case hardened article, as the pin 9 (Fig. 12) is conventionally indicated at 36 while the shading 37 (Fig. 22) indicates the soft interior or backing. It will be understood that the part 37 is no stronger than the original blank 5 (Fig. 7) while, to permit 30 the said several cold pressing operations, the said blank 5 must have been formed from steel containing not more than .15% carbon and having physical properties, substantially as follows:—

|    |                                 |       |
|----|---------------------------------|-------|
| 30 | Elastic limit pounds per square |       |
|    | inch                            | 36000 |
|    | Reduction of area               | 55%   |
|    | Elongation in two inches        | 30%   |

35 Such a steel responds only slightly to heat treatment and cannot be materially increased in strength, hardness or toughness beyond the properties indicated by the above figures. It follows, therefore, since 40 the pin 9 (Fig. 12), when case hardened, cannot be relied upon to possess added strength merely because of its said thin hardened shell 36, the walls of the said pin must be correspondingly thicker than the 45 walls of the pin 13 (Fig. 6) and there will be a similar difference in the weight of the corresponding blanks, as 5 (Fig. 7) and 11 (Fig. 4). Valuable alloy steels may thus be 50 used for the production of the machine parts provided by the present invention without unduly increasing the cost, while the reduction of weight is of itself of enormous importance in some instances, as in the case of a piston pin for internal combustion engines 55 where every effort is made to reduce the momentum of the reciprocating parts.

In Fig. 1, the numeral 4 designates a 60 brake drum formed of medium or high carbon steel and produced by the method to which this application pertains. On account of the properties of this steel as regards ductility, that is the reduction of area and elongation, it is impossible to do any commercial pressing or drawing work in the 65 cold state. If, however, this steel is heated,

as before described, it may be readily formed or drawn. Due to the superior physical properties of this steel, the finished product may be reduced in thickness and weight to only a fraction of what is required 70 in the thickness and weight of low carbon steels, formed or pressed cold, and at the same time the strength and efficiency of the product is greatly increased, it being possible to form an article thereby in one or two 75 operations while the same article would require four or five or more operations made by the cold pressing method.

Referring to Fig. 3, a forging of the rough size required for producing a brake 80 drum is shown in section at 1. In producing drop forgings, it is impossible to make the forging any nearer than the rough size of the article to be produced and after the forging is finished a considerable amount of 85 difficult and expensive machine work is necessary to turn the forging down to the required size and shape, this machine work involving a great deal of expensive labor and a wasting of at least one-half of the 90 metal in the forging. For instance, the dotted lines at 2 show the cross sectional shape of the finished brake drum which is produced from this forging, all of the metal not inclosed by these lines being wasted in 95 the machine work. Furthermore, to permit of this large amount of machine work, the forging must be softened by annealing and the finished part should be case hardened 100 to resist wear.

Referring to Fig. 2, the numeral 3 indicates a finished brake drum formed of mild or low carbon steel by the usual cold pressing process and by comparison with Fig. 1, shows the greater weight of a drum so 105 formed. It is desirable to reduce the weight of all parts of a machine, especially an automobile, unless some reason exists for desiring weight in some special part, and for this reason, a special grade of steel which 110 combines lightness and strength is best adapted for machine parts.

Wearing parts, such as brake drums, shackle bolts, piston pins and the like have occasionally been made by the cold pressing 115 process to reduce the cost of manufacture. In order that such parts could be so made, it was necessary to use a mild or soft steel having a low carbon content and a correspondingly high reduction of area and elongation, this resulting in a product which was 120 weak structurally.

Figs. 13, 14 and 15 illustrate two pairs of dies, as 29, 30, (Figs. 13 and 14), and 32, 33, (Fig. 15) which may be used for forming a 125 wheel hub from a medium or high carbon steel or steel alloy blank by the present method, the said pairs of dies being used in succession to form the blank to the finished dimensions of the wheel hub. As shown, the 130

heated blank 28, of medium or high carbon steel or steel alloy is first placed in the lower die 29, the corresponding upper die 30 co-operating therewith to form the blank into the shape shown at 31. The article 31 while still hot is then placed in the die 32, the die 33 co-operating therewith to form the finished hub 34. The finished product of the dies is now strengthened, hardened and 5 toughened throughout its entire structure by 10 heat treatment, as described in connection with the manufacture of the piston pin 13 (Fig. 6). This finished product will be considerably less in weight than a hub of like 15 size formed by the cold pressing method and at the same time will be several times as strong as the other product.

Figs. 16 to 20 inclusive show the several 20 pairs of dies required for forming a wheel hub from a mild or low carbon steel blank by the cold stamping or pressing method heretofore used; the dies of each pair operating in conjunction and the several pairs of dies being adapted to be used in succession to transform the blank into the finished wheel hub. The blank 16 of mild or low 25 carbon steel, after being first annealed, is placed in the lower die 16, the upper die 17 co-operating therewith to form the intermediate product as shown at 18, (Fig. 17). This intermediate product 18 is now annealed and then placed in the die 19 which, in conjunction with the upper die 20, forms the second intermediate product as shown 30 at 21 (Fig. 18). The intermediate product 21 is now again annealed and the several operations are repeated with respect to dies 22, 23, forming the third intermediate product 24 (Fig. 19) and dies 25, 26, forming the 35 finished hub 27 (Fig. 20) which is afterward carbonized or case hardened to give it a hardened thin shell upon its surface.

It should be noted that the finished product provided by the present invention may 40 have nearly six times the strength of products formed from the low carbon or mild steel by the cold pressing process. For this reason, articles formed by the present method, need only weigh a fraction of the 45 weight required in corresponding articles which are cold pressed from mild steel. A comparison of Figs. 1 and 2 serves to illustrate the reduction in weight made possible by the use of lighter stock for the production 50 of articles in accordance with the present invention. The finished product thus combines strength, resistance to wear and lightness.

By a comparison of Figs. 1 and 3 the advantages obtained by the invention over the 55 forging process will be readily seen as this process not only saves considerable material but also a great amount of expensive labor. Forging of such parts as the brake drums 60 shown by dotted lines in Fig. 3 has been

found impractical, owing to the enormous waste of material and the expensive machine work required to finish the product and the usual method of producing articles of this character has been by the cold pressing 70 method although, to afford the required strength, the finished product must be considerably heavier than is desirable, as is illustrated by a comparison of Fig. 2 with Fig. 1.

It will also be understood that while the articles provided by the invention may be made from either so-called straight carbon or alloy steels the carbon content must in either case be sufficiently high to provide a 80 material which responds to heat treatment in a marked degree. It is believed that for this purpose the carbon content of both straight carbon and alloy steels used in the practice of the invention should be about 85 .30% or higher and the terms medium and high carbon steels found in certain of the appended claims are to be understood as referring preferably to such steels. While very desirable results may be secured in the 90 practice of the invention with a straight carbon steel of the analysis indicated, most excellent results are also secured by the use of a chrome-vanadium alloy steel having a 95 like carbon content.

It will be observed that in each case, the article produced, as the piston pin 13, the brake drum 4, or the wheel hub 34, is tubular or cup-shaped and that the same is formed with male and female die members, 100 as 30 and 29 (Fig. 13) by pressure applied in a direction which is normal to the plane of the original plate and parallel with the axis of the finished part. There is accordingly a drawing of the metal by which desirable structural characteristics peculiar to articles so formed are obtained in the finished product.

We claim as our invention:

1. A uniformly hardened cup-shaped or 110 tubular machine wearing part of medium or high carbon steel hot pressed to substantially finished form and size from a flat plate of the said steel and hardened by heat treatment.

2. A uniformly hardened cup-shaped or 120 tubular machine wearing part of medium or high carbon alloy steel hot pressed to substantially finished form and size from a flat plate of the said steel and hardened by heat treatment.

3. A uniformly hardened cup-shaped or 125 tubular machine wearing part of medium or high carbon chrome steel hot pressed to substantially finished form and size from a flat plate of the said steel and hardened by heat treatment.

4. The method of producing hardened 130 cup-shaped or tubular machine parts which consists in heating a flat sheet or plate of

5 medium or high carbon steel or steel alloy to a temperature at which it is readily ductile, press forming the same while hot to substantially the finished form and size of the said cup-shaped or tubular machine part between male and female die members with pressure applied in a direction normal to the plane of the original plate and thereafter hardening the part throughout by heat treatment.

10 5. The method of producing machine parts which consists in heating to a temperature of approximately 1500° F. sheet or plate steel alloy containing carbon in sufficient amount to markedly respond to heat treatment, pressing the same while so heated to substantially the finished dimensions of the said machine part, packing the same in lime or similar substance while still hot and allowing it to cool while so packed, smoothing the wearing surface of the part and then uniformly hardening and toughening the part by heat treatment.

15 6. The method of producing machine parts which consists in heating to a temperature of approximately 1500° F. sheet or plate chrome-vanadium steel alloy containing carbon in sufficient amount to markedly respond to heat treatment, pressing the

same while so heated to substantially the 30 finished dimensions of the said machine part, packing the same in lime or similar substance while still hot and allowing it to cool while so packed, smoothing the wearing surface of the part and then uniformly 35 hardening and toughening the part by heat treatment.

7. A cup-shaped or tubular machine part of medium or high carbon steel hot pressed to substantially finished form and size from 40 a flat plate of the said steel and hardened throughout by heat treatment without carbonization.

8. A cup-shaped or tubular machine part of medium or high carbon alloy steel hot pressed to substantially finished form and size from 45 a flat plate of the said steel and hardened throughout by heat treatment without carbonization.

9. A cup-shaped or tubular machine part 50 of medium or high carbon chrome steel hot pressed to substantially finished form and size from a flat plate of the said steel and hardened throughout by heat treatment without carbonization.

ARTHUR J. TOWNSEND.  
HARRY M. NAU GLE.